

## UNITED STATES PATENT OFFICE

2,306,667

## ALLOY

Albert A. Smith, Jr., Metuchen, N. J., assignor to  
 American Smelting and Refining Company,  
 New York, N. Y., a corporation of New Jersey

No Drawing. Application February 13, 1942,  
 Serial No. 430,805

## 2 Claims. (Cl. 75—166)

This invention relates to lead alloys and more particularly to lead-tin-silver alloys. The alloy products of the invention are especially useful as solders but may be utilized for other purposes where it is desired to employ a metal having the physical characteristics of the lead alloys as hereinafter described.

Lead-silver solders have been known for many years but, because of their relatively high melting temperatures and poor spreading properties, they have not been extensively used. I have discovered, however, that by alloying tin with the lead-silver alloys the aforementioned disadvantages are substantially overcome while certain beneficial properties of the binary alloy are retained.

Broadly speaking, the present invention or discovery may be said to provide a ternary alloy of lead, tin and silver having certain highly advantageous physical properties. In the following table there is listed some of the significant physical characteristics of these alloys which have been determined. For comparison, corresponding test values are shown for some conventional tin-lead and silver-lead solders. Carefully standardized testing technique was employed in each instance to obtain the comparative test results shown:

TABLE  
*Some properties of soft solders*

| Composition per cent |    |      | Liquidus<br>°C. | Tensile<br>strength<br>psi | Bond<br>strength<br>of lapped<br>joints psi | Spread<br>of $\frac{1}{4}$ gr.<br>in sq. in. | Creep rate in per cent per year<br>at 30° C. |         |         |         |
|----------------------|----|------|-----------------|----------------------------|---------------------------------------------|----------------------------------------------|----------------------------------------------|---------|---------|---------|
| Pb                   | Sn | Ag   |                 |                            |                                             |                                              | 200 psi                                      | 400 psi | 600 psi | 800 psi |
| 60                   | 40 | —    | 238             | 5660                       | 6270                                        | 1.30                                         | 10.9                                         | 92      | 300     | —       |
| 97.5                 | —  | 2.5  | 304             | 4980                       | 3740                                        | 0.19                                         | 0.10                                         | 0.15    | —       | 0.50    |
| 95                   | —  | 5    | 375             | 4915                       | 4340                                        | 0.20                                         | 0.18                                         | 0.22    | —       | 0.45    |
| 95                   | —  | 5    | 312             | 4800                       | 4000                                        | 0.22                                         | —                                            | —       | —       | —       |
| 92.5                 | 5  | 2.5  | 309             | 4860                       | 4300                                        | 0.30                                         | —                                            | —       | —       | —       |
| 90                   | 10 | —    | 298             | 4850                       | 4960                                        | 0.27                                         | 2.5                                          | 12      | —       | —       |
| 87.75                | 10 | 2.25 | 1 290           | 4950                       | 5000                                        | 0.41                                         | —                                            | 2.3     | 8.0     | —       |
| 80                   | 20 | —    | 275             | 4940                       | 5680                                        | 0.37                                         | 6.7                                          | 18.7    | —       | —       |
| 78                   | 20 | 2    | 1 267           | 5620                       | 5550                                        | 0.57                                         | —                                            | —       | —       | —       |
| 70                   | 30 | —    | 267             | 5390                       | 5770                                        | 0.83                                         | 10                                           | 50      | —       | —       |
| 68                   | 30 | 1    | 1 251           | 5810                       | 5620                                        | 0.86                                         | —                                            | 4       | 20      | —       |

<sup>1</sup> Determined in this investigation from cooling curves.

NOTE.—Bond and spread tests were made on copper sheet. Tensile and creep tests were made on chill cast strips of the alloys.

The ternary alloys of lead-tin-silver offer a variety of solders which have somewhat higher melting points than the ordinary 40-60 (Sn-Pb) solder but exhibit good spreading and bond strength properties. Silver added to low-tin solders decrease the liquidus temperature from 6 to 8° C. and markedly improves the spreading properties without appreciably affecting the bond strength.

to 30% tin, 0.5% to 2.5% silver with the balance of the alloy composition being made up substantially all of lead.

50 2. A relatively low melting point alloy composition which consists principally of lead, tin and silver, said constituents approximating 5% tin, 2% silver and the balance substantially all lead.

**Disclaimer**

2,306,667.—*Albert A. Smith, Jr.*, Metuchen, N. J. ALLOY. Patent dated Dec. 29, 1942. Disclaimer filed Oct. 27, 1949, by the assignee, *American Smelting and Refining Company*.

Hereby enters this disclaimer to claim 2 of said patent.  
[Official Gazette December 20, 1949.]